

Dec. 15, 1925.

1,565,367

H. HOWARD

ELECTROLYTIC PROCESS FOR THE PRODUCTION OF COPPER CARBONATE

Filed Aug. 29, 1924



Henry Howard Inventor

By Byrnes Townsend & Bruckenstein

Attorneys.

## UNITED STATES PATENT OFFICE.

HENRY HOWARD, OF CLEVELAND, OHIO, ASSIGNOR TO THE GRASSELLI CHEMICAL COMPANY, OF CLEVELAND, OHIO, A CORPORATION OF OHIO.

## ELECTROLYTIC PROCESS FOR THE PRODUCTION OF COPPER CARBONATE.

Application filed August 29, 1924. Serial No. 735,023.

To all whom it may concern:

Be it known that I, HENRY HOWARD, a citizen of the United States, residing at Cleveland, in the county of Cuyahoga and 5 State of Ohio, have invented certain new and useful Improvements in Electrolytic Processes for the Production of Copper Carbonate, of which the following is a specification.

10 This invention relates to an electrolytic process for the production of copper carbonate.

In an application filed March 24, 1924, Serial Number 701,507, in the name of 15 Frederick F. Hunt, is described a process for the production of copper carbonate involving the electrolysis of a solution containing a carbon dioxide supplying agent, specifically sodium bicarbonate, and an electrolyte, specifically sodium sulfate, using anodes of copper and cathodes of any suitable material enclosed in diaphragms, the carbonation of the electrolyzed solution to regenerate the sodium bicarbonate, the separation of copper carbonate from the solution, and the re-use of the solution in a 25 cyclical manner.

In the course of research in this connection I have found that salts other than sodium sulfate may serve as the electrolyte and that the carbonation of the solution may be carried out in several ways other than as specifically described in said application, and more particularly that by using an alkali 30 metal chlorate, specifically sodium chlorate, as the electrolyte and by carbonating the solution within the electrolyte cell the process is improved with respect to current efficiency, yields of the copper carbonate 35 product from a given expenditure of power, even solution of the anodes, and simplification of the apparatus and procedure without, so far as I have found, any off-setting disadvantages.

40 In the following description of a preferred procedure in accordance with my invention reference is made to the accompanying drawing on which the essential parts of the apparatus and the movement of the materials are indicated diagrammatically and by means of legends.

A solution containing 80 grams of sodium bicarbonate and 220 grams of sodium chlorate in 5000 cubic centimeters of water

is continuously circulated through the electrolytic cell containing anodes of copper and cathodes of any suitable material, for instance, copper, the latter enclosed in diaphragms of for instance cotton filter cloth, and through a suitable device such as 55 a filter or settling tank for the removal of copper carbonate and back to the electrolytic cell. In the cell the solution is subjected to electrolysis, using a current density of about 60 11.5 amperes per square foot of anode surface, and to carbonation by the introduction of carbon dioxide gas. The solution in the electrolytic cell may be at about room temperature, say 70° to 100° F. Outside the 65 cell the solution is separated from copper carbonate, for instance by filtration, and returned to the cell. The rate of circulation of the solution must be sufficient to carry the copper carbonate formed and held in 70 suspension out of the cell. This depends to some extent upon the size and shape of the 75 cell and may be assisted by agitation of the electrolyte within the cell to prevent the copper carbonate from settling. The rate at which carbon dioxide is supplied depends of course upon the rate at which it is used in 80 the formation of the copper carbonate. It is preferred to supply an excess of carbon dioxide and to introduce it into the cell near the bottom thereof in order to produce agitation, the undissolved carbon dioxide being recovered and re-introduced along with the 85 fresh supply.

The foregoing process is capable of considerable variation with respect to the concentration of the solution, the relative quantities of bicarbonate and chlorate, current density, temperature, etc., without departing from my invention. The carbonation 90 may be accomplished otherwise than by the introduction of carbon dioxide directly into the solution in the electrolytic cell during the electrolysis. For instance, the solution may be electrolyzed for a period and then the passage of current stopped and carbon dioxide introduced, these two operations being repeated alternately and successively or a small portion of the solution may be 95 continuously circulated from the cell through a carbonator and back into the cell, while another portion is being withdrawn from the cell, filtered and returned to the 100 cell.

The invention therefore is not limited to the specific procedure described but includes such obvious variations thereof as are embraced by the appended claims.

8 I claim:—

1. Process for the electrolytic production of copper carbonate comprising subjecting a solution containing a carbon dioxide supplying agent and an electrolyte to electrolytic action in the presence of a copper anode, carbonating said solution during the electrolysis thereof, and removing copper carbonate from the electrolyzed solution.

2. Process for the electrolytic production of copper carbonate comprising subjecting

a solution containing a soluble bicarbonate and an alkali metal chlorate to electrolysis in the presence of a copper anode, carbonating the solution, and removing copper carbonate therefrom.

3. Process for the electrolytic production of copper carbonate comprising subjecting a solution containing sodium bicarbonate and sodium chlorate to simultaneous carbonation and electrolysis in the presence of a copper anode, and separating copper carbonate from the solution.

In testimony whereof, I affix my signature.

HENRY HOWARD.

20

25